

June 3, 1930.

A. R. ROWE

1,761,494

HOT TOP

Filed Sept. 6, 1928



Fig. 1.



Fig. 3.



Fig. 2.

Fig. 5.



Fig. 4.



Fig. 9.



Fig. 6.



Fig. 10.



Fig. 7.



Fig. 11.



Fig. 8.



Fig. 12.

INVENTOR.  
A. R. ROWE

BY J. S. NEWTON  
ATTORNEYS.

## UNITED STATES PATENT OFFICE

ANDREW R. ROWE, OF MIDLAND, PENNSYLVANIA

## HOT TOP

Application filed September 6, 1928. Serial No. 304,296.

This invention relates to improvements in hot tops and has for an object the provision of means for decreasing the amount of piping ordinarily formed in iron ingots.

5 My improvement may be used in connection with a refractory hot top open at its top and bottom but provided with a refractory loose bottom or the improvement may be used without such a hot top to decrease the piping in the ingot.

Another object of the invention is to improve the facilities for handling hot tops and for cheapening their manufacture without lessening their efficiency.

15 With these and other objects in view which will appear as the description proceeds, I will now describe my invention in connection with the accompanying drawings in which:

20 Fig. 1 represents a plan view of one form of hot top;

Fig. 2 is a cross section of the hot top shown in Figure 1, and a cross section of the top of the mold showing the hot top after it 25 has been seated on the top of the iron in the mold;

Fig. 3 is a cross section of the hot top and upper portion of the mold showing the position of the parts after an additional pouring of iron when the parts are in the position shown in Figure 2;

Fig. 4 is a view of the loose bottom for the hot top;

Fig. 5 is a view of a very much shorter hot top than the one shown in Figures 2 and 3;

Fig. 6 is a view showing a kind of hot top that is proposed to be used in my invention;

Fig. 7 is a view showing a part of the hot top of Figure 6 with a portion broken away;

Fig. 8 is a view of the under side of the hot top shown in Figure 6;

Fig. 9 is a view showing a modified form of hot top of Figure 6;

Fig. 10 is a view showing the use of a part of the hot top shown in Figure 9;

Fig. 11 is a perspective view of the hot top shown in Figure 10;

Figure 12 is another modified form of the hot top shown in Figure 11, and

Figure 13 is a bottom view of the hot top shown in Figure 12.

1 is a mold of ordinary construction. In 55 the practice of my invention I pour into the mold the melted iron 2 until the top has reached a desirable point near the top of the mold. The ordinary ladle, not shown, is then moved on to another mold or a series of molds and an attendant, after the melted iron is poured into the mold, sets the hot top 3 in the top of the mold so that its bottom rests on the melted top of the iron ingot. The hot top 3 being ordinarily 60 of refractory material, is lighter than the iron and will rest on the top as shown in Figure 2.

I may then place the loose fitting bottom 4 in the hot top and after the ladle has been 70 moved to other molds, it is brought around a second time and the iron poured into the hot top 3 of Figure 2. The melted metal at its top having frozen around the hot top 3 holds it firmly in place while the 75 second pouring of metal raises the top of the melted iron to some convenient point as shown in Figure 3 carrying with it the loose bottom 4 to the position shown in Figure 3. In this position the ingot is allowed 80 to cool and ordinarily it will be found that the piping at the top of the metal in the mold, which may have assumed a position such as shown in Figure 6, has been obliterated in the mold and the shape of the top 85 of that portion of the metal above the top of the mold will be as indicated in Figure 3.

Instead of using a deep hot top as shown in Figure 3, my improvement permits the 90 use of a hot top such as shown in Figure 5 which will, however, function very much as the hot tops shown in Figures 2 and 3.

The bottom 4 of the hot top is loose in the same and can rise in the hot top as the metal 95 is poured onto the bottom and since the bottom is lighter than the metal, the metal will run through the holes 5 in the bottom and around the edges of the bottom and get under the same and raise it to the top of the 100

hot top. By my improved method and apparatus I have been enabled to reduce the piping in the ingot from fifteen to thirty percent of the piping as it ordinarily exists without my improved apparatus and method.

Instead of using the hot tops as shown in Figures 1 to 5, I may use what might be called a refractory cover 8 shown in Figures 6 and 8. This cover may conveniently be made with flanges 9 and 10 at its bottom and a thin portion 11 within the flanges. After the metal is poured into the mold as indicated in Figure 6, I insert the cover 8 in the mold. The cover is preferably made smaller than the interior top of the mold leaving a space 12. When placed on top of the melted metal, the flanges 9 and 10 will sink down somewhat into the metal and the metal will rise in the space 12 and freeze the cover onto the metal. I then, by a sharp blow of an instrument, break away the thin portion 11 and pour a second time some metal into the mold and since the metal is heavier than the broken fragments of the cover, it will fill the piping indicated in Figure 6 and bring the metal up to a position shown as for example in Figure 7, the piping indicated at 13 in Figure 6 having been obliterated by the second pouring as indicated in Figure 7 and the cover frozen to the metal. After the second pouring of the metal, it is preferable to cover the broken away part by a separate block 35 similar to the block 16 of Figure 9 or 20 of Figure 12.

Instead of using the one-piece cover as shown in Figure 8 and breaking away the thin portion 11, I may use the two-piece cover shown in Figure 9 in which 14 is a block preferably of refractory material having a hole 15 therein. 16 is a separate block of material large enough to cover the hole 15. After filling the mold with the molten metal to a height as indicated in Figure 9, I set on top of the metal the block 14 and after an interval of time more metal is poured into the mold to obliterate the piping 13' the metal rising, for example, to the position shown in Figure 10. While the metal is still melted, I then place the block 16 over the opening 15 and allow the metal to cool before removing the covers 14 and 16.

In Figure 13 I show a modification of the block 14 of Figures 10 and 11. This block has a flange 18 and a hole 19. This block is manipulated in the same way as the one shown in Figures 9 and 10. That is to say, the metal is poured into the mold until it reaches a position as shown in Figure 12. The block 20, shown in Figure 12, is then set on top of the molten metal and more metal poured through the hole 19 until the piping at the top of the metal is obliterated and a second block 21 is placed over the hole 19 as shown in Figure 12 and allowed to remain until the metal freezes.

In all the modifications, the metal is first poured into the molds until it reaches any desirable height and the hot top or cover placed on top of the melted metal. The ladle from which the metal is poured is then moved to other molds and finally brought back and more metal poured through the hot top or cover as hereinbefore indicated, and allowed to freeze.

By the practice of my invention I have been enabled to reduce the percentage of piping in the upper part of the ingot, from twenty-five to fifty per cent.

What I claim as new is:

1. Process for reducing the piping in ingots comprising partially filling the mold with metal, then placing on top of the metal a refractory cover that will partially sink into the metal, then allowing the metal to freeze around the cover, then removing a part of the cover to expose the top of the metal and pouring a fresh supply of melted metal, allowing it to pass under a portion of the refractory cover and into the recipient piping below the bottom of the cover to obliterate any preformed piping.

2. The process of reducing the piping in metal ingots comprising partially filling a mold, covering the metal with a cover, portions of which sink into the metal and are held when the metal freezes on top, removing part of the covering after the metal has frozen around the lower portions of the cover and pouring in a fresh supply of molten metal to obliterate the preformed piping under the cover.

3. The process of reducing the formation of piping in the top of metallic ingots comprising filling a mold with the metal to a predetermined height, partially covering the metal with a heat insulating cover that will slightly sink into the top of the melted metal, then allowing the metal to slightly freeze around the cover and after the metal has frozen around the submerged portion of the cover, removing a part of the cover to expose a part of the top of the metal and pouring in a fresh supply of metal, then recovering the exposed metal with a heat insulating portion to retain the heat while the metal is finally cooling.

4. A hot top for a mold comprising a normally horizontal cover portion and vertically extending side portions smaller than the interior of the mold and composed of material lighter than the metal so that the lower portion of the vertically extending side portions will sink into the metal in the mold sufficiently to be held firmly to the metal after it is partially frozen, said horizontal portion being adapted to be easily

separated from the vertically extending portions to expose the top of the metal.

5. A hot top comprising a cover portion and projections extending below the cover and enough smaller than the mold to allow the metal to rise around the lower part of said projections, the cover proper being adapted to be easily separated from said downwardly extending portions to allow

10 metal to be poured into the mold and rise within the downwardly extending portions.

6. A hot top for a metal mold comprising a cover with a flange at the bottom of the cover the cover fitting loosely in the mold 15 and being sufficiently heavy to cause the flange to sink into the molten metal and be held in the mold when the metal partially freezes, the central portion of the hot top being easily separated from the flanged portions to allow metal to be poured into the 20 surrounding flanged portions.

In testimony whereof I hereunto affix my signature.

ANDREW R. ROWE.

25

30

35

40

45

50

55

60

65